

## UNITED STATES PATENT OFFICE

2,137,147

RUST OR CORROSION PREVENTING  
MATERIAL OR LUBRICANTEric Rose Styles, Minoco Wharf, West Silvertown,  
London, England, assignor to Silvertown Lu-  
bricants Limited, London, EnglandNo Drawing. Application February 23, 1937, Se-  
rial No. 127,316. In Great Britain February 4,  
1936

10 Claims. (Cl. 87—9)

This invention relates to solid, semi-liquid or liquid materials having lubricating and/or rust or corrosion-resisting or preventing properties.

The object of the present invention is to provide a stable lubricant and/or material adapted to afford protection against rust or corrosion, which is substantially innocuous or relatively harmless to rubber, rubber-like masses or rubber compounds, with the advantage that the lubricant or material may be freely used in situations where it is difficult or impossible to avoid its coming into contact with rubber or the like or with materials incorporating it, vulcanized or otherwise. It is a further object of the invention to provide 10 a substantially anhydrous lubricant having the above mentioned qualities.

The invention is based upon the observation that no appreciable deleterious action on rubber and rubber-like masses results from treatment 20 with castor oil in the absence of petroleum hydrocarbons and free fatty acids and that castor oil assumes desirable physical characteristics when incorporated with an oil soluble metal soap.

According to the invention, a material suitable 25 for use as a lubricant or corrosion-resisting coating material comprises castor oil and a metal soap (other than an alkali metal soap) and is substantially free from free fatty acids and petroleum hydrocarbons.

Also in accordance with the invention, a material suitable for use as a lubricant or corrosion-resisting coating material is prepared by incorporating castor oil with a metal soap (other than an alkali metal soap), preferably with the 30 employment of the minimum heat necessary to liquefy the soap, and neutralizing free acid present by treatment with a basic substance.

Freedom from free fatty acid may be ensured by treatment of the castor oil with any suitable 40 basic substance in quantity at least equivalent to the free fatty acid content, a preferred basic substance being the carbonate of the metal of the soap employed, especially if the quantity of free fatty acid is relatively large.

In carrying out the invention, it is preferred 45 to employ the heavy metal soaps and in particular the lead soaps. The lead soaps produce an unctuous, sticky, free-flowing grease with excellent properties as an extreme pressure lubri- 50 cant.

The amount of the metal soap employed is desirably adjusted according to the desired viscosity or consistency of the material, a convenient range of concentration being from about 8% to about 30% of the castor oil.

Other substances which are free from petroleum hydrocarbons may be added to the material for the purpose of modifying its properties, for example neutral wool grease may be included to increase the anti-corrosive properties. As, however, it appears that such additional substances are not without some deleterious effect on rubber, even in the case of neutral wool grease, it is desirable to limit the addition to not more than 10% and, preferably, not more than about 2½% 10 of the lubricant; while if it is desired to obtain the maximum inertness towards rubber in the composition of the invention such additional substances should be avoided.

In carrying the invention into effect according 15 to one convenient method for producing a soft lubricant having a melting point in the range 75° to 100° C., castor oil is heated together with from 8 to 10% of lead stearate, the temperature employed being sufficient only to melt the lead 20 soap completely, e. g. 125° C., since the use of higher temperatures may result in discoloration of the product. Any acidity in the mixture is neutralized by addition of the appropriate 25 amount of lead carbonate.

A lubricant of medium hardness may be prepared by proceeding in the manner described above and increasing the lead stearate content to 15% of the castor oil. A hard lubricant is obtained when an amount of lead stearate of from 30 25 to 30% is employed.

As lead stearate has a higher melting point than most common lead soaps, the substitution of other lead soap for the lead stearate in the examples given above will usually result in a lubricant of lower melting point.

Having now described my invention, what I claim as new and desire to secure by Letters Patent is:—

1. A material having lubricating and corrosion-resisting qualities and suitable for use in contact with rubber, consisting of castor oil and a metal soap, other than an alkali metal soap, and a basic substance capable of neutralizing the free fatty acids present in the oil. 40

2. A material having lubricating and corrosion-resisting qualities and suitable for use in contact with rubber, consisting of castor oil and a heavy metal soap in amount from 8% to 30% of the amount of castor oil, and a basic substance capable of neutralizing the free fatty acids in the oil. 50

3. A material as claimed in claim 1 wherein the metal soap is a lead soap.

4. A material as claimed in claim 1 wherein the metal soap is lead stearate.

5. A material as claimed in claim 2 wherein the heavy metal soap is a lead soap.
6. A material as claimed in claim 2 wherein the heavy metal soap is lead stearate.
- 5 7. A material having lubricating and corrosion-resisting qualities and suitable for use in contact with rubber, formed essentially from castor oil, a heavy metal soap and a basic substance capable of neutralizing free fatty acids in amount at least equivalent to free fatty acid present in the oil.
- 10 8. A material having lubricating and corrosion-resisting properties and suitable for use in con-
- tact with rubber, formed essentially from castor oil, a heavy metal soap, and the carbonate of the heavy metal of the soap in amount at least equivalent to free acid present in the oil.
9. A material having lubricating and corrosion 5 resisting properties and suitable for use in contact with rubber, formed essentially of castor oil, a lead soap and lead carbonate in amount at least equivalent to free fatty acid present in the oil.
- 10 10. A material as claimed in claim 9 wherein 10 the lead soap is lead stearate.

ERIC ROFE STYLES.